

[72] Inventor David M. Eissenberg  
Oak Ridge, Tenn.  
[21] Appl. No. 826,102  
[22] Filed June 20, 1969  
[45] Patented Dec. 15, 1970  
[73] Assignee The United States of America as  
represented by the United States Atomic  
Energy Commission.

[54] **METHOD FOR PROMOTING DROPOWSE  
CONDENSATION ON COPPER AND COPPER  
ALLOY CONDENSING SURFACES**  
5 Claims, 1 Drawing Fig.

[52] U.S. Cl. .... 165/1,  
165/110, 165/133  
[51] Int. Cl. .... F28f 13/18  
[50] Field of Search. .... 165/1, 133,  
110

[56]

## References Cited

## OTHER REFERENCES

Drew et al., TB, The Conditions for Drop-Wise Condensation of Steam, Transactions of American Institute of Chemical Engineers, Vol. 31, No. 4, 12/25/1935, pp. 613 and 614, TP 1.A6 (now Chemical Engineering)

Hampson, H. Heat Transfer During Condensation of Steam, Engineering, 8/17/1951, p. 221, TA 1.E55

Primary Examiner—Albert W. Davis, Jr.  
Attorney—Roland A. Anderson

**ABSTRACT:** A method for promoting dropwise condensation on copper and copper alloy condensing surfaces is provided. Clean metallic surface finishes are developed and preserved on which steam condensate forms in droplets as a result of maintaining a concentration of a few parts per million of CO<sub>2</sub> at the condensing surface. The CO<sub>2</sub> may be carried by the condensing vapor or injected directly into the condensing chamber.



PATENTED DEC 15 1970

3,547,185



INVENTOR.  
*David M. Eissenberg*  
BY  
*Ronald A. Goodman*  
ATTORNEY.

**METHOD FOR PROMOTING DROPWISE  
CONDENSATION ON COPPER AND COPPER ALLOY  
CONDENSING SURFACES**

**BACKGROUND OF THE INVENTION**

The invention described herein relates generally to surface condensers and more particularly to a method of promoting dropwise condensation of steam on copper and copper alloy surfaces. It was made in the course of, or under, a contract with the U. S. Atomic Energy Commission.

When a condensing surface is coated with a substance which prevents the condensate from wetting the surface, the vapor will dense condense in drops, or dropwise, on the condensing surface rather than in the form of a continuous film. Such dropwise condensation, as opposed to the continuous film or filmwise condensation, has long been considered desirable because of the relatively large heat transfer coefficients associated therewith. Heat transfer coefficients achieved under dropwise condensation conditions have been found to be from four to eight times as high as with filmwise condensation.

It has been found that condenser tubes plated with noble metals such as silver, gold and platinum promote dropwise condensation under long term conditions with high purity water. Such materials are prohibitively expensive, however, and as a result have not been considered commercially practical as plating materials for promoting dropwise condensation. Certain organic materials such as waxes and silicones have also been observed to promote dropwise condensation but are also considered impractical in that they do not form a permanent coating and cannot be economically replenished. Plastic coatings such as polytetrafluoroethylene and polyparaxlylene are known to promote dropwise condensation, but have proven undesirable for that purpose in that at practical coating thicknesses they act as insulators and thereby offset any gains achieved as a result of the dropwise condensation.

It is, accordingly, a general object of the invention to provide a means for promoting dropwise condensation on a condensing surface formed of or plated with an inexpensive commercially available metal.

Other objects of the invention will be apparent from an examination of the following description of the invention and the appended drawing.

**SUMMARY OF THE INVENTION**

In accordance with the invention, a method for promoting dropwise condensation on copper and copper alloy condensing surfaces is provided. Clean metallic surfaces accompanied by dropwise condensation are developed and conserved by maintaining a concentration of a few parts per million of CO<sub>2</sub> at the condensing surface. Dropwise condensation is thus achieved without the need for forming or coating the condensing surfaces with expensive metals having inherent nonwetting characteristics or providing them with semipermanent organic surface coatings.

**BRIEF DESCRIPTION OF THE DRAWING**

The FIG. is a graph of heat transfer coefficients as a function of time for a condensing system operated in accordance with the invention.

**DETAILED DESCRIPTION**

Applicant has discovered that copper and copper base alloy condensing surfaces have operated in an unexpected manner in the presence of very small concentrations of CO<sub>2</sub> in the condensing vapor. Concentrations of a few parts per million of CO<sub>2</sub> in the condensing vapor have been found to cause the condensing surfaces to operate in the dropwise condensing mode. Dropwise condensation is considered highly desirable because of the high heat transfer coefficients associated therewith as compared to the coefficients achieved in the filmwise condensation which normally occurs with uncoated copper and copper alloy condensing surfaces.

Although the exact mechanism of the invention is not known with certainty by applicant, it is believed that the CO<sub>2</sub> provided in accordance with the invention dissolves in the condensate to form a weak carbonic acid solution. The carbonic acid dissolves copper oxide as it forms on the condensing surface, thereby maintaining the surface clean and suitable for dropwise condensation. Although other explanations may be found to account for the effect discovered by applicant, such explanations will in no way affect the scope of applicant's invention which is limited only by the appended claims. In practice, others may use applicant's invention by providing CO<sub>2</sub> concentrations as taught herein without regard to its exact operating mechanism.

15 The invention will be more specifically illustrated by means of the following examples:

**EXAMPLE I**

A sample of 1-inch outside diameter commercial copper tubing was installed in a test condenser. A small patch, about 1 inch square, was cleaned with emery paper to remove surface oxide. Steam at 215° and 15.5 p.s.i.a. from the plant steam system was admitted to the condenser. Within 24 hours, the cleaned area was condensing in dropwise fashion while the remainder of the tube condensed filmwise. After 3 days, the entire tube was condensing dropwise. The system was shut down and air admitted. Upon restarting the system, the entire tube surface was observed to revert to filmwise condensation. The tube subsequently returned to dropwise condensation within a few hours after restarting. Noncondensables in the steam were analyzed as 80 percent CO<sub>2</sub>, 18 percent N<sub>2</sub> and less than 2 percent O<sub>2</sub> with a trace of H<sub>2</sub>. The total concentration of noncondensables in the steam was about 5 parts per million.

**EXAMPLE II**

A 90-10 copper-nickel condenser was treated in the manner described in example I. This tube exhibited the same conversion from filmwise to dropwise condensation as the commercial copper tubing of example I.

**EXAMPLE III**

In another test, a 304 stainless steel condenser tube was 45 tested in the manner described in example I. The stainless steel tube failed to convert from filmwise to dropwise condensation and the test was terminated after one week. EXAMPLE IV

In another series of tests, a special steam generator was used 50 to provide better control over the kind and concentration of noncondensables present in the steam. The steam generator used deaerated, demineralized water for conversion to steam. A 90-10 copper-nickel tube specimen was placed in the condenser and steam from the generator admitted. Condensation on the tube specimen was observed to be filmwise for several days. The tube was observed to have a dark copper oxide color during this portion of EXAMPLE test. Carbon dioxide was then admitted to the steam feed stream in an amount estimated to be a few parts per million. After a few hours the dark copper oxide color began to turn to a patchy pink color and condensation was observed to convert from the filmwise to the dropwise mode. During subsequent shutdown periods, the condenser tube was observed to darken but upon each startup the color improved and filmwise condensation converted to dropwise. A later addition of hydrogen to the CO<sub>2</sub>-steam mixture had no observable effect on the results achieved with CO<sub>2</sub> above.

**EXAMPLE V**

In another run, hydrazine was bled into the steam along with CO<sub>2</sub>. The final result was the same as in example IV except that the oxide coating appeared to clear somewhat faster. It is thus postulated that hydrazine or other reducing agents may 75 be desirable additives along with CO<sub>2</sub> during the initial startup

of a condensing unit in order to accelerate the transition to dropwise condensation. EXAMPLE VI

In another test, a 3-inch outside diameter doubly fluted 90-10 copper-nickel tube was tested for an extended period in a vertical tube evaporator test assembly. Plant steam, having the same noncondensable content as described in example I, was used as the steam supply. Heat transfer coefficients were determined immediately after startup and again when the oxide film on the tube began to lighten in color and dropwise condensation was first observed. Further heat transfer coefficient determinations were made over a 6-day period until condensation appeared to be entirely dropwise. The heat transfer coefficients obtained during the test run are plotted in the FIG. The heat transfer coefficients plotted in the FIG. are nominal, overall, average coefficients based on nominal outside tube circumferences and nominal temperature differences between the condensing steam and coolant liquid discharged from the tube as inferred from pressure measurements, and they include tube-wall resistances. The slight reduction in overall heat transfer coefficients which occurred after the seventh day resulted when a 4.9 weight percent NaCl solution was substituted for the evaporator feedwater. Although the improvement in heat transfer is good, it is noted that this particular tube design is superior to conventional tube design and therefore the improvement over conventional tubes is even greater. Good performance of the tube was sustained under test conditions over a 6-day period whereas in the prior art, the performance of all condenser tubes has been observed to deteriorate after a short period due to surface oxide buildup.

Although the invention is especially desirable for use in large condensers such as are used and/or planned for use in desalination plants of the evaporator type, it may be used in any heat transfer device in which heat is removed from a vapor through a wall, causing the vapor to condense on the

wall. Various means may be used for maintaining the desired concentration of CO<sub>2</sub> at the condensing surfaces including the injection of CO<sub>2</sub> directly into the condenser chamber or letting it be carried by the condensing vapor. It is also noted that the CO<sub>2</sub> concentration in a condenser should be kept as low as possible consistent with the condenser tubes operating in a dropwise condensation mode. Concentrations exceeding that minimum value sufficient to bring about and maintain dropwise condensation are undesirable since the presence of any noncondensable in the condenser tends to lessen its efficiency. Thus, although a value of about 5 parts per million has been found to be workable by applicant under test conditions, lesser concentrations may be adequate during steady state operation or in other systems where very little oxygen is present in the condenser.

I claim:

1. In a heat transfer system wherein water vapor is condensed by contacting it with a copper base cooling surface, the improved method for promoting dropwise condensation of said vapor on said cooling surface comprising maintaining a sufficient concentration of CO<sub>2</sub> in the water vapor adjacent to said cooling surface to cause dropwise condensation to occur.
2. The improved method of claim 1 wherein said concentration of CO<sub>2</sub> in the water vapor adjacent to said cooling surface is about 5 parts per million.
3. The improved method of claim 1 wherein said cooling surface is a condenser tube.
4. The improved method of claim 1 wherein a reducing agent is added to said water vapor during the initial startup period of said heat transfer system to accelerate the transition from filmwise to dropwise condensation.
5. The improved method of claim 4 wherein said reducing agent is hydrazine.